

## 1

3,384,479

## COLUMBIUM-BASE ALLOYS

Winston H. Chang, Cincinnati, Ohio, assignor to General  
Electric Company, a corporation of New York  
No Drawing. Filed July 8, 1965, Ser. No. 470,560  
3 Claims. (Cl. 75—174)

## ABSTRACT OF THE DISCLOSURE

Columbium-base alloys consisting essentially of, by weight, about 30% W, 0.05—0.12% C, 0.5—6.0% of Ti, Zr, or Hf, or combinations thereof have been found to have very high creep and tensile strengths at elevated temperatures and are ductile and fabricable at low temperatures.

This invention relates to high strength workable columbium-base alloys, and more particularly to such alloys which are capable of possessing significant tensile ductility at room temperature.

Over the past decade, many improvements have been made in columbium-base alloys resulting in higher strength combined with workability, oxidation resistance and other desirable factors. Naturally, further significant improvements that can be made in these areas will continue to be desirable. However, it has come to be accepted that significant increases in high temperature strength are generally accompanied by diminishing or disappearing low temperature ductility and its concomitant characteristic—workability.

Although increasing amounts of highly refractory solid solution alloy additives were found to be useful in increasing strength in the lower alloy ranges such as up to about 10 or 15%, it was generally expected that significantly higher amounts of solute metals such as tungsten would be quite harmful to ductility and workability. Indeed, it was considered by some that increases beyond 20% tungsten in carbide strengthened columbium-base alloys would not result in increased strengthening. (Percentages herein are by weight except where indicated otherwise.)

It is a principal object of the present invention to provide columbium-base alloys having significantly higher levels of strength at elevated temperatures such as 2400° F. to 3000° F. than previously available in combination with workability and low temperature ductility in a fabricated condition.

Another object of the invention is to provide such alloys that also possess useful oxidation resistance so that they might be used in oxidizing atmospheres with appropriate coatings, and might be useful in nonoxidizing atmospheres containing small amounts of residual oxidizing impurity gases even without coatings.

Briefly stated, the present invention in one aspect provides columbium-base alloys consisting essentially of, by weight, about 30% W, 0.05—0.12% C, 0.5—6.0% total reactive metal selected from the group consisting of Ti, Zr and Hf and combinations thereof, the balance essentially all columbium and residual impurities. Aside from carbon, other interstitial elements including oxygen and nitrogen may be useful in stabilizing precipitates, or, alternatively, they might be considered as residual impurities having no great effect on the properties of the alloy, de-

## 2

pending on the situation. Other specific embodiments of the invention include such alloys in which the titanium content is about 0.5% and the zirconium content is about 0.8—1%, with 0.05—0.1% carbon, and an alloy with 0.5—1.0% zirconium and 0.5—0.1% carbon.

Experimental work leading to the present invention included the study of two alloys designated therein as Cb-1 and Cb-2. The nominal and analyzed compositions of these two alloys are presented in Table I below.

TABLE I.—CHEMICAL ANALYSES

| Alloy | Item <sup>1</sup> | Analysis, Weight Percent |       |      |       |        |        |
|-------|-------------------|--------------------------|-------|------|-------|--------|--------|
|       |                   | W                        | Ti    | Zr   | C     | O      | N      |
| Cb-1  | [N]               | 30.0                     | ..... | 1.0  | 0.1   | .....  | .....  |
|       | [A]               | 29.66                    | ..... | 0.83 | 0.058 | 0.0103 | 0.0440 |
| Cb-2  | [N]               | 30.0                     | 5.0   | 1.0  | 0.1   | .....  | .....  |
|       | [A]               | 29.96                    | 1.93  | 0.86 | 0.058 | 0.0101 | 0.0295 |

<sup>1</sup> N=nominal; A=analyzed.

Cb-1 and Cb-2 were consolidated by pressing together well-blended metal powders in the proportions in the nominal compositions to form electrodes which were then sintered and vacuum-arc melted. Based on heat-treatment results of as-cast materials, the ingots were extruded at 3750° F. for Cb-1 and 3500° F. for Cb-2. Both ingots were extruded, jacketed in molybdenum cans, at a ratio of about 9:1, resulting in significant hot-work with incipient recrystallization. Swaging was then performed on the Cb-1 extruded bar at 2750° F. for a 50% reduction in cross section, followed by swaging for a total of 93% reduction in area (from extrusion) at 500° F. The same swaging treatment was successfully performed on extrusions of both alloys following aging at 2700° F. for one hour.

The one-hour complete recrystallization temperatures were determined to be 3200° F. for Cb-1 and 2900° F. for Cb-2.

My studies have shown that the Cb-1 alloy contains a face-centered-cubic (FCC) phase (Zr, Cb, W)C which may also contain substantial amounts of oxygen and nitrogen as the stable precipitate below about 3000° F. Above that temperature, Cb<sub>2</sub>C and ZrO<sub>2</sub> also exist. Apparently due to the additional presence of Ti, alloy Cb-2 contains as its precipitate the FCC phase (Zr, Cb, Ti, W)C exclusively, except for small amounts of ZrO<sub>2</sub>. The Ti content and especially the ratio of (Ti+Zr)/C seem to suppress the formation of Cb<sub>2</sub>C.

Aging studies were performed on specimens of swaged Cb-1 and Cb-2 solution treated at 3500° F. and then aged for one hour at various temperatures in the range of 1500—3000° F. Maximum hardness aging peaks occur at about 2100° F. for Cb-1 and 1750° F. for Cb-2. The age hardening of Cb-1 appears to be accompanied by dissolution of the Cb<sub>2</sub>C phase and precipitation of FCC (Zr, Cb, W)C phase. Within the 2000—2250° F. range of peak hardening, however, the precipitating FCC phase could not be discerned under optical examination. In alloy Cb-2, the (Zr, Cb, Ti, W)C precipitated directly from the matrix in the absence of any pre-existing Cb<sub>2</sub>C.

These studies indicate that carbide dispersion strengthening is most effective in these alloys at temperatures below about 2200° F., although some strain-induced precipitation may persist up to 250° F. Thus, solution strengthening becomes more effective and more necessary for retaining strength at higher temperatures. I have discovered that about 30% tungsten in combination with the stated amounts of carbide-precipitating additives results in con-

siderably stronger alloys than previously available possessing workability and low temperature ductility in an as-worked condition and when stress-relieved.

Tensile testing of specimens in various heat-treated conditions has shown that alloy Cb-1 possesses ample room-temperature ductility after one-hour stress relief at 2500° F., either directly swaged or aged before being swaged, and alloy Cb-2 possesses such ductility after stress-relief treatment at 2200° F.

tion than in a stress-relief condition, particularly in alloy Cb-1.

An alloy of the prior art with which Cb-1 can be compared is alloy F-48, having a nominal composition of 15% W, 5% Mo, 1% Zr, 1% C, the balance columbium. Table III presents a comparison of the tensile properties of Cb-1 and F-48 showing that Cb-1 is considerably stronger at elevated temperatures, while still retaining superior ductility even at room temperature.

TABLE III.—TENSILE PROPERTY COMPARISON CB-1 VS. F-48

| Alloy | Swaging Temp., °F. | Stress Relief Temp., °F. | Test Temp., °F. | Tensile Strength, K s.i. | Elongation, percent |
|-------|--------------------|--------------------------|-----------------|--------------------------|---------------------|
| F-48  | 2,200-2,100        | 2,000                    | 78              | 149.0                    | 19                  |
|       |                    |                          | 2,000           | 81.4                     | 21                  |
|       |                    |                          | 2,500           | 48.7                     | 21                  |
| Cb-1  | 2,750-2,500        | 2,500                    | 3,000           | 15.6                     | 14                  |
|       |                    |                          | 78              | 139.3                    | 24                  |
|       |                    |                          | 2,000           | 72.0                     | 20                  |
|       |                    |                          | 2,500           | 51.8                     | 29                  |
|       |                    |                          | 3,000           | 24.7                     | 101                 |

Table II presents data on the tensile properties of Cb-1 directly swaged and as swaged after having been aged at 2750° F. for one hour. The column on heat treatment involves three treatments for one hour: S.R. 1 is a stress

20 Table IV compiles tensile properties of the Cb-2 alloy as swaged after having been aged at 2750° F. for one hour. S.R. means stress relief for one hour at 2200° F., and R<sub>x</sub> means recrystallization at 2900° F. for one hour. As it did for Cb-1, recrystallization of Cb-2 raises the ten-

TABLE IV.—TENSILE PROPERTIES OF CB-2 ALLOY

| Test Temp., °F. | Heat Treatment    | Tensile Strength, K s.i. | 0.2% Yield Strength, K s.i. | Elongation, percent | Reduction in Area, percent |
|-----------------|-------------------|--------------------------|-----------------------------|---------------------|----------------------------|
| 78              | S.R.              | 155.0                    | 145.3                       | 13.0                | 12.4                       |
|                 |                   | 150.8                    | 143.0                       | 17.6                | 45.8                       |
|                 |                   | 150.7                    | 143.0                       | 19.1                | 46.2                       |
| 250             | R <sub>x</sub>    | 133.0                    | 132.8                       | 0                   | 0                          |
|                 |                   | 115.3                    | 111.3                       | 7.4                 | 7.5                        |
|                 |                   | 106.3                    | 95.5                        | 26.1                | 71.8                       |
| 500             | (R <sub>x</sub> ) | 101.0                    | 92.6                        | 27.7                | 66.3                       |
|                 |                   | 93.3                     | 78.3                        | 20.7                | 75.6                       |
|                 |                   | 95.5                     | 73.3                        | 17.0                | 62.7                       |
| 1,000           | (S.R.)            | 108.5                    | 72.8                        | 18.2                | 75.6                       |
|                 |                   | 89.4                     | 68.3                        | 20.1                | 64.0                       |
|                 |                   | 69.4                     | 64.4                        | 10.2                | 76.8                       |
| 1,500           | (R <sub>x</sub> ) | 87.0                     | 57.0                        | 16.4                | 62.9                       |
|                 |                   | 45.8                     | 41.6                        | 30.9                | 86.7                       |
|                 |                   | 43.8                     | 38.6                        | 27.9                | 87.2                       |
| 2,000           | (S.R.)            | 45.7                     | 42.3                        | 26.2                | 50.3                       |
|                 |                   | 17.5                     | 17.2                        | 75.2                | 63.5                       |
|                 |                   | 18.3                     | 18.1                        | 69.0                | 67.7                       |

relief at 2200° F., S.R. 2 is a stress relief at 2500° F., and R<sub>x</sub> is a recrystallization treatment at 3200° F.; K s.i. means thousands of pounds per square inch.

sile transition temperature (in this case to about 300° F.) and results in somewhat higher tensile strength than that of the stress-relieved condition.

TABLE II.—TENSILE PROPERTIES OF CB-1 ALLOY  
[A. Directly Swaged]

| Test Temp., °F.                       | Heat Treatment | Tensile Strength, K s.i. | 0.2% Yield Strength, K s.i. | Elongation, percent | Reduction in Area, percent |
|---------------------------------------|----------------|--------------------------|-----------------------------|---------------------|----------------------------|
| 78                                    | S.R. 1         | 124.8                    | 122.7                       | 0.5                 | 0.5                        |
|                                       |                | 130.2                    | 125.0                       | 2.6                 | 3.0                        |
|                                       |                | 139.3                    | 121.7                       | 24.3                | 41.7                       |
| 500                                   | S.R. 2         | 106.5                    | 92.6                        | 31.1                | 81.1                       |
|                                       |                | 102.3                    | 77.2                        | 19.2                | 78.2                       |
|                                       |                | 95.0                     | 73.7                        | 21.7                | 82.2                       |
| 1,000                                 | S.R. 2         | 72.0                     | 65.8                        | 20.3                | 88.0                       |
|                                       |                | 55.3                     | 53.0                        | 32.1                | 99.0                       |
|                                       |                | 52.0                     | 46.5                        | 31.7                | 99.5                       |
| 2,000                                 | S.R. 2         | 51.8                     | 48.0                        | 29.1                | 99.0                       |
|                                       |                | 41.3                     | 33.2                        | 27.5                | 99.6                       |
|                                       |                | 24.7                     | 17.4                        | 101.2               | 99.4                       |
| [B. Aged at 2750° F. 1 Hour + Swaged] |                |                          |                             |                     |                            |
| 78                                    | S.R. 1         | 129.5                    | 128.5                       | 0.7                 | 0                          |
|                                       |                | 145.5                    | 125.8                       | 18.7                | 16.7                       |
|                                       |                | 138.0                    | 126.0                       | 8.8                 | 8.4                        |
| 500                                   | R <sub>x</sub> | 149.8                    | 149.7                       | 0.3                 | 0                          |
|                                       |                | 112.7                    | 94.1                        | 24.4                | 56.4                       |
|                                       |                | 119.7                    | 104.3                       | 27.5                | 47.0                       |
| 1,000                                 | R <sub>x</sub> | 105.0                    | 80.4                        | 20.5                | 79.1                       |
|                                       |                | 106.0                    | 80.8                        | 23.2                | 55.2                       |
|                                       |                | 95.8                     | 74.3                        | 19.4                | 83.2                       |
| 1,500                                 | R <sub>x</sub> | 132.3                    | 78.4                        | 16.9                | 11.4                       |
|                                       |                | 76.0                     | 68.6                        | 19.6                | 89.1                       |
|                                       |                | 111.2                    | 69.0                        | 10.6                | 10.0                       |
| 2,000                                 | R <sub>x</sub> | 58.4                     | 54.7                        | 24.4                | 93.6                       |
|                                       |                | 59.2                     | 54.2                        | 23.9                | 91.5                       |
|                                       |                | 73.2                     | 64.5                        | 11.1                | 20.5                       |
| 2,700                                 | R <sub>x</sub> | 44.8                     | 34.8                        | 33.2                | 98.6                       |
|                                       |                | 60.0                     | 48.8                        | 16.9                | 32.5                       |
|                                       |                | 27.9                     | 25.9                        | 67.1                | 96.5                       |
| 3,000                                 | R <sub>x</sub> | 31.3                     | 28.4                        | 49.2                | 59.4                       |

Although recrystallization raises the ductile-to-brittle transition temperature, it is accompanied by strain-induced precipitation, resulting in considerably higher strengths at temperatures above 1000° F. in the recrystallized condi-

Likewise, alloy Cb-2 can be compared with prior art alloy F-50, having a nominal composition of 15% W, 5% Mo, 1% Zr, 5% Ti, 0.1% C, the balance columbium.

The same strength superiority accompanied by room-temperature ductility retention over F-50 is found with Cb-2 as was found with Cb-1 over F-48.

29,000 p.s.i., corresponding to a 100-hour strength-to-density ratio of 78,000 inches (0.371 lb./in.<sup>3</sup> nominal). In addition to room-temperature ductility, rupture ductility

TABLE V.—TENSILE PROPERTY COMPARISON Cb-2 VS. F-50

| Alloy     | Swaging Temp., °F. | Stress Relief Temp., °F. | Test Temp., °F. | Tensile Strength, K. s.i. | Elongation, percent |
|-----------|--------------------|--------------------------|-----------------|---------------------------|---------------------|
| F-50----- | 2,200-2,100        | 1,900                    | 78              | 145.7                     | 25                  |
|           |                    |                          | 2,000           | 65.3                      | 29                  |
|           |                    |                          | 2,500           | 29.0                      | 14                  |
|           |                    |                          | 3,000           | 11.6                      | 20                  |
| Cb-2----- | 2,750-2,500        | 2,200                    | 78              | 150.7                     | 19                  |
|           |                    |                          | 2,000           | 69.4                      | 19                  |
|           |                    |                          | 2,400           | 45.8                      | 31                  |
|           |                    |                          | 3,000           | 17.5                      | 75                  |

All tensile testing of Cb-1 and Cb-2 alloys was performed in vacuum (except at room temperature) at a 20 nominal strain rate of 0.05/minute. The stress-relieved tensile specimens were of the button-head type having a gauge section of 0.16 inch diameter and 1.1 inch length. The recrystallized specimens had a smaller gauge section of 0.125 inch diameter by 0.33 inch length to assure the 25 complete removal of surface defects.

Stress-rupture testing was performed at 2400° F. to establish the 100-hour strength. The rupture specimens were identical to what was used for tensile testing, and

of the Cb-1 was characterized by about 20% elongation and 80% reduction of area. Due in part to overaging and incipient recrystallization, the 100-hour strength of Cb-2 at 2400° F. was found to be about 14,500 p.s.i. The conformity of the rupture data to the Larson-Miller parametric relationship suggests that the 2000° F. 100-hour strength of Cb-1 and Cb-2 should be about 50,000 p.s.i. and 40,000 p.s.i. respectively.

Satisfactory oxidation-resistant characteristics of Cb-1 and Cb-2 were found and are tabulated in Table VII

TABLE VI.—CREEP-RUPTURE DATA ON STRESS-RELIEVED ALLOYS

| Alloy     | Condition <sup>1</sup> | Stress, K.s.i. | Life, Hrs. | MCR, Percent/hr. | Elongation, Percent | Reduction in Area, Percent |
|-----------|------------------------|----------------|------------|------------------|---------------------|----------------------------|
| Cb-1----- | A-----                 | 35.0           | 14.32      | 0.97             | 11.1                | 77.0                       |
|           |                        | 30.0           | 30.0       | 0.70             | 17.7                | 78.4                       |
|           | B-----                 | 30.0           | 137.72     | 0.046            | 20.4                | 77.7                       |
|           |                        | 30.0           | 54.29      | 0.122            | 22.0                | 77.0                       |
|           |                        | 27.5           | 124.05     | 0.047            | 21.7                | 81.0                       |
| Cb-2----- | B-----                 | 35.0           | 1.76       | -----            | 23.2                | 75.5                       |
|           |                        | 30.0           | 3.70       | -----            | 22.3                | 59.4                       |
|           |                        | 20.0           | 5.34       | 1.67             | 18.5                | 69.1                       |
|           |                        | 17.5           | 28.64      | 0.44             | 47.5                | 82.0                       |
|           | B-----                 | 15.0           | 71.82      | 0.02             | 41.2                | 82.7                       |

<sup>1</sup> A = directly swaged and stress relieved; B = aged, swaged, and stress relieved.

testing was conducted by direct loading in a radiation-heated furnace evacuated by an ion pump to a vacuum of 10<sup>-8</sup> torr. Data obtained are presented in Table VI above.

The data were consistent and well correlated by the 50 Larson-Miller parametric relationship of  $P = T(15 + \log t)$  where T is temperature in degrees Rankine and t is hours. The 100-hour strength of Cb-1 was found to be about

below. Alloy Cb-2 is significantly superior to alloy Cb-1, due in part to the titanium content of Cb-2.

Although the present invention has been described with respect to certain embodiments, it will be understood by those skilled in the art that certain changes, omissions and substitutions may be made within the spirit and scope of the invention as defined in the appended claims.

TABLE VII.—OXIDATION DATA OF CB-BASE ALLOYS <sup>1</sup>

| Temp., °F. | Time, hrs. | Weight Gain, mg. cm. <sup>-2</sup> |       | Depth of Hardening, mils side |       | Metal Loss, mils side |       |
|------------|------------|------------------------------------|-------|-------------------------------|-------|-----------------------|-------|
|            |            | Cb-1                               | Cb-2  | Cb-1                          | Cb-2  | Cb-1                  | Cb-2  |
| 1800-----  | 1          | 6.0                                | 3.2   | 17                            | 9     | 0.3                   | 0     |
|            | 3          | 23.5                               | 8.2   | 25                            | 15    | 1.4                   | 0     |
|            | 8          | 93.1                               | 18.6  | 32                            | 17    | 7.2                   | 1     |
|            | 16         | 201.4                              | 25.8  | 38                            | 20    | 28.5                  | 1.5   |
|            | 16         | 123.8                              | 28.8  | -----                         | ----- | -----                 | ----- |
|            | 24         | 300.0                              | 28.6  | 35                            | 20    | 52.5                  | 1.9   |
| 2100-----  | 24         | 30.3                               | ----- | -----                         | ----- | -----                 | ----- |
|            | 24         | 305.0                              | ----- | -----                         | ----- | -----                 | ----- |
|            | 1          | 15.6                               | 12.3  | 25                            | 12    | 1.3                   | 0.13  |
|            | 3          | 27.5                               | 19.1  | 33                            | 15    | 3.9                   | 1.0   |
|            | 8          | 49.6                               | 34.5  | 40                            | 21    | 4.2                   | 2.0   |
|            | 16         | 74.8                               | 46.9  | 53                            | 28    | 6.6                   | 3.3   |
| 2400-----  | 24         | 96.7                               | 60.4  | 65                            | 32    | 9.0                   | 4.0   |
|            | 50         | 169.2                              | 89.6  | >97                           | 51    | 17.6                  | 7.1   |
|            | 100        | 250.1                              | 133.5 | >88                           | 67    | 27.0                  | 10.9  |
|            | 1          | 32.4                               | 28.0  | 30                            | 15    | 2.8                   | 1.6   |
|            | 3          | 67.4                               | 51.9  | 46                            | 25    | 6.2                   | 3.4   |
|            | 8          | 137.2                              | 115.4 | 70                            | 35    | 12.9                  | 6.3   |
|            | 16         | 230.0                              | 146.5 | >91                           | 45    | 24.4                  | 11.3  |
|            | 24         | 312.9                              | 198.0 | >75                           | 55    | 40.0                  | 15.4  |

<sup>1</sup> Terminal air tests unless otherwise indicated.

<sup>2</sup> Continuous weight-gain air test.

What I claim as new and desire to secure by Letters Patent of the United States is:

1. A columbium-base alloy consisting essentially of, by weight, about: 30% W, 0.05-0.12% C, 0.5-6.0% total reactive metal selected from the group consisting of Ti, Zr and Hf and combinations thereof, the balance essentially all columbium and residual impurities. 5

2. A columbium-base alloy consisting essentially of, by weight, about: 30% W, 0.05-0.1% C, 1-5% Ti, 0.8-1% Zr, and the balance essentially all columbium and residual impurities. 10

3. A columbium-base alloy consisting essentially of, by weight, about: 30% W, 0.5-1.0% Zr, 0.05-0.1% C, the balance essentially all columbium and residual impurities.

## References Cited

## UNITED STATES PATENTS

|           |         |              |       |        |
|-----------|---------|--------------|-------|--------|
| 2,973,261 | 2/1961  | Frank        | ----- | 75-174 |
| 3,056,672 | 10/1962 | Clark        | ----- | 75-174 |
| 3,113,863 | 12/1963 | Chang et al. | ----- | 75-174 |

## FOREIGN PATENTS

|         |        |               |
|---------|--------|---------------|
| 889,099 | 2/1962 | Great Britain |
| 923,225 | 4/1963 | Great Britain |

CHARLES N. LOVELL, Primary Examiner.